# EUROPEAN PATENT SPECIFICATION

(11) **EP 0 041 540 B1**
(45) Date of publication and mention of the grant of the patent: **23.01.1985**
(21) Application number: 81900104.1
(22) Date of filing: 10.11.1980
(51) Int. Cl.: G03C 1/72

(54) **COLOR IMAGING SYSTEM**
FARBPHOTOGRAPHISCHES ABBILDUNGSSYSTEM
SYSTEME PHOTOGRAPHIQUE EN COULEUR

(30) Priority: 07.12.1979 US 101144; 07.12.1979 US 101197
(43) Date of publication of application: 16.12.1981
(73) Proprietor: MINNESOTA MINING AND MANUFACTURING COMPANY, St. Paul, Minnesota 55133-3427 (US)
(72) Inventor: WINSLOW, John M., St. Paul, MN 55133 (US); GATZKE, Kenneth G., St. Paul, MN 55133 (US)
(74) Representative: Bowman, Paul Alan
(86) International application number: US8001506
(87) International publication number: WO8101757

## Description

A layer comprising 1) an oxidizing ion and 2) leuco dye or bleachable dye in a binder is useful as either an imaging layer or as a heat-bleachable antihalation layer. The antihalation layer is particularly useful in photothermographic systems where the development temperatures acts to bleach the dye.

It is known from Chemical Abstracts, Vol. 82, No. 20, page 488, Abstract 132141 z to provide a thermographic system comprising a leuco dye, and a nitrate or nitrite as a latent colour developer which releases an oxidizing agent upon heating to oxidize the leuco dye to a coloured form. In Derwent Patents Report, Vol. 79, No. 17, Section C4 (J79009062) is disclosed a heat sensitive copying material comprising colour developing agent, reducing agent and nitric acid or a nitrate, in which colour is developed by exposure to IR radiation.

It has been found that the addition of an acid to an imageable layer comprising a leuco dye or a bleachable dye and a nitrate salt, can reduce the concentration of nitrate ion required for satisfactory colour formation (by oxidation of a leuco dye) or bleaching (by oxidation of a bleachable dye) upon heating the layer.

According to the present invention there is provided an imageable layer comprising a polymeric binder, and within said binder a leuco dye or bleachable dye, and a nitrate salt, the nitrate ion of which being present in a ratio of at least 0.1 moles/mole of dye, characterised in that an acid is present within the binder and said nitrate salt in said binder is capable of liberating a sufficient quantity of oxidizing agent selected from HN0₃, NO, N0₂ and N₂0₄ when heated to up 200°C for 60 seconds to oxidize said bleachable dye to a different colour or colourless state or oxidize said leuco dye to a coloured state.

The present invention may be practiced in any polymeric binder system having the necessary active ingredients therein. These ingredients comprise leuco dyes or bleachable dyes and a, preferably non-dye-reactive (as herein defined), nitrate salt. The active agents also include an acid which supplies hydrogen ion. A binder material containing these ingredients can be colourised or decolourised locally by heating portions of the binder layer or generally decolourised by heating the entire layer. The presence of the acidic material accelerates the decolourisation phenomenon.

### The Binder

Any polymeric binder may be used in the practice of the present invention. The pH of the resin has been found to affect only the speed of the discolourising effect, If the speed is not important, any resin may be used. Organic polymeric resins are generally preferred, more particularly thermoplastic resins although thermoset resins may be used. Where speed is more important, the more acidic resins should be used to decrease the pH and increase the rate of oxidation or decolorizing. Such resins as polyvinyl acetals, polyesters, polyvinyl resins, polyvinylpyrolidone, polyesters, polycarbonates, polyamides, polyvinyl butyral, polyacrylates, cellulose esters, copolymers and blends of these classes of resins, and others have been used with particular success. Natural polymeric materials such as gelatin and gum arabic may also be used. Where the proportions and activities of dyes and nitrate ion require a particular developing time and temperature, the resin should be able to withstand those conditions. Generally it is preferred that the polymer not decompose or lose its structural integrity at 93°C (200°F) for 30 seconds, and more preferred that it not decompose or lose its structural integrity at 127°C for 30 seconds and most preferred that it withstand 144°C (290°F) for 60 seconds.

Beyond these minimal requirements, there is no criticality in the selection of a binder. In fact, even transparency and translucency are not required, although they are desirable. Where, for example, the polymer with the bleachable dye is itself an opaque white, the thermally treated area will become white and the non-treated areas will remain the color of the dye.

The binder serves a number of additionally important purposes in the constructions of the present invention. The imageable materials are protected from ambient conditions such as moisture. The consistency of the coating and its image quality are improved. The durability of the final image is also significantly improved.

### The Nitrate Salt

Nitrate salts are themselves well known. They may be supplied as various compounds forms, but are preferably provided as a metal salt, and most preferably provided as a hydrated metal salt. Other ions which are ordinarily good oxidizing ions such as nitrite, chlorate, iodate, perchlorate, periodate, and persulfate do not provide comparable results. Extremely active oxidizing agents, such as iodate, even used in relatively smaller proportions to prevent complete and immediate oxidation or decolorization of dyes do not perform nearly as well as nitrate ion compositions. The performance of nitrate is so far superior to any other ion that it is apparently unique in the practice of the present invention. While some of the better oxidizing ions other than nitrate can only produce modest differences between the maximum optical density (Dₘₐₓ) and the minimum optical density (Dₘᵢₙ) or produce high Dₘᵢₙ values even in their best constructions, the better constructions with nitrate ions can have a Dmax in excess of 1.0 and a Dₘᵢₙ below 0.10.

Most means of supplying the nitrate ion into the composition are satisfactory. E.g., metal salts, acid salts, mixtures of acids and salts, and other means of supplying the ion are useful. For example, nitrates of zinc, cadmium, potassium, calcium, zircon, nickel, aluminum, chromium, iron, copper, magnesium, lead, and cobalt, ammonium nitrate, and cerous ammonium nitrate have been used.

The nitrate salt component of the present invention must be present in a form within the imaging layer so that HN0₃, NO, N0₂, or N₂0₄ will be provided within the layer when it is heated to a temperature no greater than 200°C for 60 seconds and preferably no greater than 160°C for 60 or most preferably 30 seconds. This may be accomplished with many different types of salts, both organic and inorganic, and in variously different types of constructions.

The most convenient way of providing such thermal oxidant providing nitrate salts is to provide a hydrated nitrate salt such as aluminum nitrate nonahydrate (AI(NO₃)_{2'}9H₂0). This salt, when heated in a binder, will generate HN0₃, NO, NO_{Z} and/or N₂0₄ in various amounts. The binder should not be at such a high pH that the liberated nitric acid would be imediately neutralized as this would adversely affect the oxidizing capability of the system. PH levels above 8.5 may in many cases completely prevent oxidation. It is therefore desired that the nitrate salt containing layer have an acidic environment such as a pH less than 7.5, preferably equal to or less than 7.0, and more preferably equal to or less than 6.5.

In addition to hydrated nitrate salts, non-hydrated salts in an acidic environment are also capable of providing HN0₃, NO, N0₂, and/or N₂0₄ in sufficient quantities to provide the oxidizing capability necessary for practice of the present invention. Ammonium nitrate, for example, does not enable good oxidation in a layer having a pH of 8.0 or higher, but when a moderate strength organic acid such as phthalic acid is added to lower the pH to below 7.0, a quite acceptable imaging system is provided.

Beside the inorganic types of salts generally described above, organic salts in non-alkaline environments are also quite useful in the practice of the present invention. In particular, nitrated quaternary ammonium salts such as quanadinium nitrate work quite well in acid environments, but will not provide any useful image at alkaline pH levels or 8.0 or higher.

It is believed that an alkaline environment causes any oxidizing agent (e.g., HN0₃, NO, N0₂ and/or N₂0₄) which is liberated from the nitrate salt to be preferentially reacted with hydroxy ions or other neutralizing moieties so as to prevent oxidation of the dyes. For this reason it is preferred to have the environment of the nitrate salt acidic, effectively at a pH no greater than 7.0 and more preferably less than 6.5.

One other consideration should be given in the selection of the nitrate salt and that is the choice of a salt in which the cation is non-reactive with the dye. Non-reactive salts are defined in the practice of the present invention as those salts the cations of which do not spontaneously oxidize the dyes that they are associated with at room temperature. This may be readily determined in a number of fashions. For example, the dye and a non-nitrate (preferably halide) salt of the cation may be codissolved in a solution. If the salt oxidizes the dye spontaneously (within two minutes) at room temperature, it is a reactive salt. Such salts as silver nitrate, in which the cation is itself a strong oxidizing agent, is a reactive salt. Cerric nitrate is also reactive, while hydrated cerrous nitrate is not.

Preferred salts are the hydrated metal salts such as nickel nitrate hexahydrate, magnesium nitrate hexahydrate, aluminum nitrate nonahydrate, ferric nitrate nonahydrate, cupric nitrate trihydrate, zinc nitrate hexahydrate, cadmium nitrate tetrahydrate, bismuth nitrate pentahydrate, thorium nitrate tetrahydrate, cobalt nitrate hexahydrate, gadolinium or lanthanum nitrate nonahydrate, mixtures of these hydrated nitrates and the like. Non-hydrated or organic nitrates may be admixed therewith.

Organic nitrates are also quite useful in the practice of the present invention. These nitrates are usually in the form of quaternary nitrogen containing compounds such as guanadinium nitrate, pyridinium nitrate, and the like. Nitrated dyes will also be useful, but again, they must be used in an environment which will not neutralize any liberated HN0₃, NO, N0₂, and/or N_{Z}O₄.

It is necessary to have at least 0.10 moles of nitrate ion per mole of dye. It is more preferred to have at least 0.30, more preferably at least 0.50 moles of ion per mole of dye. Even amounts of from 1.0 to 100 moles of nitrate ion per mole of dye have been found useful. With dyes having relatively higher oxidation potentials, more nitrate is desirable.

### Dyes

It is believed that essentially all leuco dyes (as defined herein) and bleachable dyes are useful in the present invention. With some constructions it may be desirable to select dyes which have an oxidation potential of less than or equal to +1.0. The dyes may be selected from any class of dyes. These classes include but are not limited to 1) methines, 2) indamines, 3) anthraquinones, 4) triarylmethanes, 5) benzylidenes, 6) monoazos, 7) oxazines, 8) azines, 9) thiazines, 10) xanthenes, 11) indigoids, 12) oxonols, 13) cyanines, 14) merocyanines, 15) phenols, 16) naphthols, 17) pyrazolones, and others, of which most are classified by the Colour Index System.

The measurement of oxidation potentials is well known to the ordinary skilled artisan. The measurements in the present invention are taken by measuring the voltage and current transferred between a carbon and a platinum electrode through the appropriate solution. 0.1 M lithium chloride in anhydrous methanol with 1 to 10 millimoles/liter of the appropriate dye was the standard solution used in the measurements given herein with a saturated calomel electrode.

Leuco dyes are colorless dyes which when subjected to an oxidation reaction form a colored dye. These leuco dyes are well known in the art (e.g., The Theory of the Photographic Process, 3rd Ed., Mees and James, pp. 283-4, 390-1, Macmillion Co. N.Y.; and Light-Sensitive Systems, Kosar, pp. 367, 370-380, 406 (1965) Wiley and Sons, Inc., N.Y.) and U.S. Patent 3,974,147. Amongst the known leuco dyes are leuco malachite blue, leuco malachite green, leuco crystal violet, and 1(2-(1,3,3-trimethylindolyl))-2-(p-morpholinylphenyl)ethene. Only those dyes which can be converted to colored dyes by oxidation are useful as leuco dyes in the practice of the present invention. Acid or base sensitive dyes such as phenolphthalein are not useful in the present invention unless they are also oxidizable to a colored state. Indicator dyes would only form transient images or would be too sensitive to changes in the environment.

The leuco dye should be present as at least 0.3% by weight of the binder, preferably as at least 1 % by weight of the binder, and most preferably as from 2 to 10% or more by weight of the binder.

The proportions of nitrate salt and leuco dye should preferably be such that on heating the layer at 127°C for 30 seconds there is at least an optical density of 0.2 obtained, although with a mechanical viewing of the image or heating to a higher temperature, a lower optical density is useful. Depending upon the relative ease of colorizing the particular dye selected, the relative proportion of nitrate ion to dye may vary. At least 0.1 moles of nitrate ion per mole of dye is required in the practice of the present invention. At least 0.3 or 0.5 moles of nitrate per mole of dye is more preferred, and at least 0.7 or 0.9 moles of nitrate per mole of dye is most preferred.

It is preferred to have sufficient bleachable dye in the binder prior to imaging so that at least 15% of incident radiation (including ultraviolet and infrared) in a 50 nm range would be absorbed through a 0.5 mm layer of binder and dye. Preferably at least 75% of the incident radiation in a 20 nm range would be absorbed. These ranges must of course be chosen within the spectral absorption region of the particular dye, but such absorption in any portion of the spectrum is useful. In terms of weight percentages, it would be preferred to have at least 0.30% by weight of dye as compared to the binder. Preferably, at least 0.50% by weight of dye to binder is desired and most preferably there should be at least 1% by weight of dye to binder in the layer up to 10% or more.

The bleachable dyes which have been specifically shown to work in the present invention include but are not limited to the following: wherein
R₂ = C₂H₅ ; C₇H₁₅ ; (CH₂)₅COOH ; C₈H₁₇ ; CH₂CH₂⌀ ; or
CH₂COOH
R₃ = H ; C₂H₅O ; or Cl R₄ = C₂H₅ ; or CH₂CH₂C₆H₅ wherein
R₂ = H ; -CH₂COOH ; or -CH₂CH = CH₂ wherein
R₁ = C₂H₅ ; n-C₃ H₇ ^{= R}₂ wherein
R₁ = H ; or -CN
R_{2 =} -CN ; or -SO₂CF₃ = R₃ wherein
R₁ = = S ;
R₂ = H ; CH₃ = R₃
R₄ = C₂H₅ ; C^{H}₂C^{H} = C^{H}₂ ; or CH₂CH₂CO₂C₂H₅
R₅ = -C₂H₅ ; -CH₂CH-CH₂ ; or -C₇H₁₅
R₆ = -CH₂COOH ; -CH₂CH = CH₂ ; or -(CH₂)₂SO₃H wherein
R₁ = -C₂H₅ ; -C₇H₁₅ ; or -CH₂CH = CH₂
R₂ = =S ; or =C(CN)₂
R₃ = -CH₃; or -C₂H₅ wherein
_{R1 =} -C₂H₅ ; -(CH₂)₂OH ; -(CH₂)₂COOH ; -CH₂COOH ; or -(CH₂)₃So₃⁻
R₂ = -C₂H₅ ; -(CH₂)₂oH ; -(CH₂)₂COOH ; -CH₂COOH ; or -CH₃
R₃ = H ; -CH₃; -SCH₃ ; or -C₂H₅
R₄ = H ; -CH₃ ; -Br ; or -N(C₂H₅)₂
R₅ = H ; -CH₃ ; or -Br wherein
R₁ =-CH₃ ; -C₂H₅ - R2 = R3 wherein
^{R}₃ = H ; Br whereinin
R₁ = H ; Cl wherein
R₁-S ; wherein
R₁ = -CH₃ ; or CH₃O-
R₂ = -C₂H₅ ; or -C₇H₁₅ wherein
R₁ = -OH ; -NH₂ ; -NHC₂H₅
R₂ = H ; -OH : -OCH₃
R₃ = H ; -OH ; or -NHC₂H₅ wherein
R₁ = H ; -CH₃ : or -C₂H₅
R₂ = H ; -C₂H₅ ; or -CH₂COOH
_{R} = =S ; or =CHNO₂ wherein in
R₁ = H ; or CH₃O-
^{R}₂ = -C₂H₅ ; -CH₂CO₂-(C₂H₅)₃N⁺H whereinin
R₁ = H ; -^{N}(^{CH}₃)₂
R₂=H; -Cl

The following two dyes cannot be conveniently classed by the Colour Index System:

These examples are not intended to represent the limits of the present invention. Any dye, and particularly those having an oxidation potential of +1.0 or less, may work in the present invention. The substituent groups and dye structure are unimportant.

The bleachable dyes of the present invention are preferably colored, that is, having absorbance in the visible portion of the electromagnetic spectrum (approximately 400 to 700 nm), but may also be colorless, having absorbance only or predominately in the infrared (700 to 1100 nm) or ultraviolet (310 to 400 nm) portions of the electromagnetic spectrum. The images where colorless dyes are used must then be viewed through a filter, by an ultraviolet sensitive apparatus, or by some enhancement technique.

There should be sufficient bleachable dye present in the layers of this invention so that transmissive optical density of at least 0.1 in the visible portions of the spectrum is obtained or at least 5% of incident colorless light (including ultraviolet or infrared) is absorbed. It is preferred that an optical density of at least 0.5 or 0.8 be obtained and most preferably that there be sufficient dye so that an optical density of at least 1.0 be obtained in the layer. With colorless dyes (e.g., ultraviolet and infrared absorbing dyes), it is preferred that at least 20% or 40% of incident radiation be absorbed and most preferably that at least 60% or 90% of the incident colorless light within a 20 nm range be absorbed.

The proportions of nitrate ion and dye should be such that on heating the layer at 127°C (260°F) for 30 seconds there is at least a 20% reduction in optical density, although with a mechanical viewing of the image, a lower reduction in optical density is useful. Depending upon the relative ease of decolorizing the particular dye selected, the relative proportion of nitrate ion to dye may vary. At least 0.1 moles of nitrate ion per mole of dye is required in the practice of the present invention. At least 0.3 or 0.5 moles of nitrate per mole of dye is more preferred, and at least 0.7 or 0.9 moles of nitrate per mole of dye is most preferred. Where the decolorizable layers of the present invention are used as antihalation layers, particularly with thermally developable imaging materials, more than a 20% reduction in optical density is usually desirable. At least 50% or 60% is preferred and at least 90% or 95% reduction in optical density is most preferred. These reductions can be measured at the development temperatures for the imaging materials, e.g., 127°C for 30 seconds or 155°C for 45 seconds.

### The Acids

The acids utilized in the present invention are acids as generally known to the skilled chemist. Organic acids are preferred, but inorganic acids (generally in relatively smaller concentrations) are also useful. Organic acids having carboxylic groups are more preferred. The acid may be present in a ratio up to 10 times the amount of the nitrate ion. More preferably it is present in amounts from 0.2 to 2.0 times the amount of nitrate ion.

In forming the dye layers or coating of the dye layers onto a substrate, temperatures should, of course, not be used during manufacture which would completely oxidize the layer. Some colorization or decolorization is tolerable, with the initial dye concentrations chosen so as to allow for anticipated color changes. It is preferred, however, that little or no dye be formed or decolorized during forming or coating so that more standardized layers can be formed. Depending on the anticipated development temperature, the coating or forming temperature can be varied. Therefore, if the anticipated development temperature were, for example, 167°C (350°F) the drying temperature could be 138°C and it would not be desirable for the layer to lose 20% of its optical density at the drying temperature in less than 4-5 minutes, although it would be tolerable by correspondingly increasing the amount of dye. Thus the preferred limitation of at least 20% reduction in optical density or absorbance of colorless light at 127°C for 30 seconds is based on the assumption of a development temperature of 127°C. For an anticipated higher or lower development temperature, the 20% reduction in optical density or absorbance should occur at that development temperature within a reasonable period of time. A reasonable development temperature range is between 82°C and 193°C and a reasonable dwell time is between 5 seconds and 5 minutes, preferably at between (105°C and 167°C and for 10 to 180 seconds, with the longer times most likely associated with the lower development temperatures. Therefore, all of the absorbance characteristics are applicable to the generally useful development range of 82°C to 193°C. Photothermographic imaging materials are well known in the art in various and sundry forms. Silver reduction systems (e.g., as disclosed in U.S. Patent. No. 3,457,075 and 3,849,049), thermal diazonium salt systems (e.g., as described in U.S. Patent No. 3,754,916), and others are examples of these systems. Typical constructions of these photothermographic systems will comprise one or two layers which constitute a photothermographic imaging system coated over a base. If the support base is transparent, the heat-bleachable layer of the present invention may be coated either between the imaging layers and the base or on the backside of the base. If coated between the base and the imaging layer, it is desirable to minimize competing reactions. This can be done, for example, by selecting polymers and solvent systems for the various layers which will not promote migration between the layers. When the base is opaque, the heat-bleachable layer must be between the imaging layers and the base. This would, of course also be true if there were more than one imaging layer.

All of this will be more thoroughly understood by consideration of the following examples:

### Examples 1-13

A three component system of the present invention was evaluated by using nickel nitrate hexahydrate, phthalic acid and a merocyanine dye of the formula The dye was provided as a solution of 0.8 g dye/100 ml of a solvent comprising 50/50 volume proportions of methanol and N-methylpyrrolidone. Three different concentrations of each ingredient were used. These ingredients were added to 2.5 g methanol and 12.5 g of a 10% by weight solids solution of polyvinylbutyral (as a binder) and methanol. The solutions were coated at 0.076 mm thickness on a polyester backing then dried for 3 minutes at 70°C. Maximum optical density (Dₘₐₓ) readings were taken. The coated sheets were then heated at 127°C for 30 seconds and the final maximum optical density (D_{f}) measured. The difference between Dₘₐₓ and D_{f} is the change in optical density (A D). The concentrations of materials and results appear in Table I.

### Examples 14-16

These examples evaluate the benefits of an acidic environment of the bleaching or decolorizing of the present invention. For this example, a dye of the structure was used in a solution having 0.8 g dyes/100 ml of solvent comprising a 50/50 volume solution of methanol and N-methyl-pyrrolidone. The coating solutions were as follows:

The acid was phthalic acid, the nitrate was nickel nitrate hexahydrate. The coating solution was prepared, coated, and dried as in Example 1, then heated for thirty seconds at 127°C (260° F). Example 14 bleached from medium blue to pale yellow, 15 became a lighter purple, and 16 became a light yellow. This shows that in the absence of an acid environment, greater concentrations of nitrate are desirable for more complete bleaching.

### Examples 17-24

These examples show the wide variety of acids which can be used in the construction and indicates that the acid functionality is not dependent upon the structure of the acid. All constructions were identical to those of Examples 14-16 except that 5.5 ml of dye and 0.05 g of nickel nitrate hexahydrate were used. The sheets were heated at 127°C for 30 seconds in an inert fluorocarbon bath. All sheets were initially a medium blue.

### Example 25

This example demonstrates the use of the heat-decolorizable layer as an antihalation backing for a photothermographic film.

A solution was prepared by dissolving 8 g of magnesium nitrate hexahydrate and 12 g of phthalic acid in 75 g of methanol. This was broken down into aliquots of 3 g of solution, to which were added 4 ml of dye solution containing 0.15 g of malachite green and 0.05 g of crystal violet in 10 ml of a 50/50 volume solution of methanol and N-methylpyrrolidone.

Crystal violet has an oxidation potential greater than +1.0 and has the structure: Acid malachite green, also used in the practice of the present invention, has the same structure except that one of the dimethylamine groups has been replaced by a hydrogen atom.

To the dye and nitrate containing solution was added 12.5 g of a solution of 15% by weight cellulose acetate, 10% methylisobutylketone, 10% methanol, and 65% acetone. The final solution was coated onto the backside of a commercially available photothermographic film (3M Dry Silver Film Type 8220) which comprises a transparent backing having an imageable layer thereon comprised of silver halide in catalytic proximity to silver behenate in a binder with a mild silver reducing agent. These materials are well described in U.S. Patent No. 3,475,075. The coating thickness was 0.076 mm (3 mils) and was dried for 3 minutes at 70°C. A photothermographic film with the antihalation backing was exposed at the same time as the sample without the backing to artificial daylight through a continuous step wedge. Both examples were then developed at 127°C for 30 seconds. The antihalation backing bleached to a pale yellow. The effect of the antihalation layer was obvious to the untrained eye. Image flare was significantly reduced.

### Example 26

The antihalation backing of the previous example was coated on transparent polyester film and dried at 70°C. The colored film was thermographically exposed imagewise in a thermographic copier ("Secretary" Copier by 3M). The film bleached in an area corresponding to the image on the original. This demonstrates the use of the films as an image producing element which, for example, could be used as a transparency for overhead projector.

There are a number of features of the present invention which should be noted. The imaging materials have excellent shelf life. They may set for months at ambient conditions and in room light without any deterioration in properties, to the degree that the dyes themselves are lighfstable. They are inexpensive to make and have a broad range of utility. No light sensitive materials need be present in the system and no external chemistry need be applied in order to develop an image. The absence of photosensitive and even thermally sensitive materials (except for whatever gives the present invention its thermally developable properties) is particularly noteworthy. No silver halides or diazonium salts are needed for light sensitivity and there is no need for the external application of toners. The present system is remarkable in its simplicity. The present system is preferably light insensitive in that exposure to light does not sensitize or desensitize the construction to any form of thermal or chemical development. That is, if the imageable layer of the present invention is exposed to light in an imagewise fashion then generally heated or generally exposed to a reducing agent, there will be no image formed corresponding to the light exposure. This is true even when the layer is laminated to a light sensitive substrate.

### Examples 27-39

Examples 1-13 were repeated for each of the following nitrate salts: Aluminum nitrate, nonahydrate, cobalt nitrate hexahydrate, zirconyl nitrate, ceric ammonium nitrate, barium nitrate, cupric nitrate trihydrate, silver nitrate, chromium nitrate nonahydrate, thorium nitrate tetrahydrate, bismuth nitrate pentahydrate, ferric nitrate nonahydrate, sodium nitrate and potassium nitrate. These systems also showed decolorizing effects. The multivalent salts tended to be significantly better than the monovalent salts, except that silver nitrate performed as well as many of the multivalent salts because of the oxidizing ability of the silver ion.

The imaging layers of the present invention may contain various materials in combination with the essential ingredients of the present invention. For example, lubricants, coating aids, antioxidants (e.g., ascorbic acid, hindered phenols, phenidone, etc. in amounts that would not prevent oxidation of the dyes when heated), surfactants, antistatic agents, mild oxidizing agents in addition to the nitrate, and brighteners may be used without adversely affecting practice of the invention.

The imaging layers of the present invention must allow reactive association of the active ingredients in order to enable imaging. That is, the individual ingredients may not be separated by impenetrable barriers within the layer, as with dispersed immiscible phases. Generally, the active ingredients are homogeneously mixed (e.g., a molecular mixture of ingredients) within the layer. They may be individually maintained in heat softenable binders which are dispersed or mixed within the layer and which soften upon heating to allow migration of ingredients, but this would require a longer development time.

As can be seen from the constructions of the examples, light sensitive or radiation sensitive components such as silver halide, photolabile halogen compounds, diazonium salts, or photooxidant compounds are not essential for the practice of the present invention. In fact, the preferred construction of the present invention is not light sensitive. That is, if the element were exposed to light in an imagewise manner prior to thermal development of the entire sheet, there would be no dramatic differential image formed. As almost all dyes fade or bleach with prolonged exposure to light, light insensitivity for the element must be defined as stated above, with the exposure being less than that capable of photobleaching the dye itself.

### Example 40

A coating composition comprising 2.0 grams phthalic acid, 0.3 grams crystal violet, 12.3 grams acetone, 15.4 grams N-methylpyrrolidone, 150 grams of 30% by weight solutions of polyvinylidine chloride in tetrahydrofuran (5%) and methylethylketone (65%) and 0.17 grams of guanidine and nitric acid in equal molar proportions was coated at 75,am wet thickness on polyester base and dried for three minutes at 75°C. Imagewise heating for forty seconds at 290°F (143°C) provided an image with a Dmln of 0.17 and a Dₘₐₓ of 0.86.

### Example 41

Each and every one of the dye structures listed above with Roman numerals was found to thermally image by bleaching in one of the following systems.

The first system tried was 3 ml of a dye solution formed by dissolving 0.1 g dye in 10 ml of a N-methylpyrrolidone/methanol (50/50 volume). To this was added 0.05 g of Ni(NO₃)₂·6H₂O and 0.05 g of phthalic acid in 2.5 g methanol. This was then combined with 12.5 g of a resin solution comprising 10% by weight cellulose acetate, 10% methylisobutyl ketone, and 80% acetone. If the dye did not bleach well when heated in this air dried composition, the proportions were varied by increasing the amount of Ni(N0₃)₂.6H₂0 and phthalic acid to 0.20 g each, increasing the cellulose acetate to 20% and the methylisobutyl ketone to 20% in the resin solution, while reducing the acetone to 60% in the resin solution. All of the dyes were shown to thermally bleach in an imagewise fashion in this manner.

### Example 42

A coating solution was prepared by dissolving 8 g of magnesium nitrate hexahydrate and 12 g of phthalic acid in 75 g of methanol. To a 3 g aliquot of this solution was added 4 ml of a dye solution containing 0.20 g of leuco malachite green in 10 ml of a 50/50 volume solution of methanol and n-methylpyrrolidone. To this leuco dye and nitrate solution was added 12.5 g of a solution of 15% by weight cellulose acetate, 10% methylisobutylketone, 10% methanol, and 65% acetone. This was coated onto clear polyethyleneterephthalate and dried below 90°C for ten minutes. Upon imagewise heating to 127°C for thirty seconds, an image was produced with a Dₘₐₓ of about 1.0 and a low D_{min'}

### Examples 43-46

Example 42 was repeated except that the magnesium salt was replaced with equimolar (based on nitrate ion) proportions of aluminum nitrate nonahydrate, nickel nitrate hexahydrate, chromium nitrate nonaydrate, and potassium nitrate (the last with 0.5 g of glycerol added to the first solution). After development as in Example 42, the nickel, aluminum, and chromium salts showed similar results with Dₘₐₓ values in excess of 0.9. The potassium salt produced a much weaker, but visible image.

### Examples 47-49

Example 42 was repeated except that the leuco malachite green was replaced by equal molar amounts of leuco crystal violet, 1(2-(1,3,3-trimethylindolyl))-2-(p-morpholinylphenyl)ethene, and the leuco dye Upon development as in Example 42, violet, red and pale blue images were respectively formed in each of the colorizable systems.

The imaging layers of the present invention may contain various materials in combination with the essential ingredients of the present invention. For example, lubricants, coating aids, antioxidants (e.g., ascorbic acid, hindered phenols, phenidone, etc. in amounts that would not prevent oxidation of the dyes when heated), surfactants, antistatic agents, mild oxidizing agents in addition to the nitrate, and brighteners may be used without adversely affecting practice of the invention.

The imaging layers of the present invention must allow reactive association of the active ingredients in order to enable imaging. That is, the individual ingredients may not be separated by impenetrable barriers within the layer, as with dispersed immiscible phases. Generally, the active ingredients are homogeneously mixed (e.g., a molecular mixture of ingredients) within the layer. They may be individually maintained in heat softenable binders which are dispersed or mixed within the layer and which soften upon heating to allow migration of ingredients, but this would require a longer development time.

## Claims

1. An imageable layer comprising a polymeric binder, and within said binder a leuco dye or bleachable dye, and a nitrate salt, the nitrate ion of which being present in a ratio of at least 0.1 moles/mole of dye, said nitrate salt in said binder being capable of liberating a sufficient quantity of oxidizing agent selected from HN0₃, NO, N0₂ and N₂0₄ when heated up to 200°C for 60 seconds to oxidize said bleachable dye to a different colour or colourless state or oxidize said leuco dye to a coloured state, characterised in that an acid is present within the binder.

2. An imageable layer as claimed in Claim 1, in which the ratio of the moles of nitrate ion to moles of dye is at least 0.5.

3. An imageable layer as claimed in Claim 1 or Claim 2, in which said acid is present within said binder in a ratio up to 10 times the amount of nitrate ion.

4. An imageable layer as claimed in any preceding claim, in which the pH of said imageable layer is less than 7.0.

5. An imageable layer as claimed in any preceding claim, in which said nitrate salt in said binder is capable of liberating said sufficient quantity of oxidizing agent when heated to up to 160°C for 60 seconds.

6. An imageable layer as claimed in any preceding claim, in which said nitrate salt comprises a metal nitrate salt.

7. An imageable layer as claimed in Claim 6, in which said nitrate salt comprises a hydrated metal nitrate salt.

8. An imageable layer as claimed in Claim 7, in which said nitrate salt is a hydrated salt of one of the group consisting of zinc, cadmium, nickel, aluminium, iron, copper, magnesium, chromium, cobalt, bismuth, lanthanum, galolinium, thorium, zirconium, and calcium.

9. An imageable layer as claimed in any preceding claim, which is light insensitive.

10. An imageable layer as claimed in any one of Claims 1 to 9, in which said dye is present in an amount of at least 0.3% by weight of the binder.

11. An imageable layer as claimed in any one of Claims 1 to 9, in which said dye is a bleachable dye present in a concentration of dye sufficient to provide a transmissive optical density of at least 0.1 in the visible region of the electromagnetic spectrum.

12. An imageable layer as claimed in any preceding claim, in which said dye is a bleachable dye, selected from methines, indamines, anthraquinones, triarylmethanes, benzylidenes, monoazos, oxazines, azines, thiazines, xanthenes, indigoids, oxonols, cyanines, merocyanines, phenols, naphthols and pyrazolones.

13. An imageable layer as claimed in any one of Claims 1 to 10, in which said dye is a leuco dye selected from leuco crystal violet, leuco malachite blue, leuco malachite green, and 1(2-(1,3,3-trimethylindolyl))-2-(p-morpholinylphenyl)-ethene.

## Revendications

1. Couche photographique comprenant un liant polymère qui contient un leucocolorant ou une matière colorante décolorable et un nitrate, l'ion nitrate étant présent dans la proportion d'au moins 0,1 mole/mole de colorant, ledit nitrate dans ledit colorant étant capable de libérer une quantité suffisante d'agent oxydant appartenant au groupe de HN0₃, NO, N0₂ et N₂0₄ quand on le chauffe jusqu'à 200°C pendant 60 secondes pour oxyder ladite matière colorante décolorable en une couleur différente ou un état incolore, ou pour oxyder ledit leucocolorant en un état oxydé, ladite couche photographique étant caractérisée en ce qu'un acide est présent dans le liant.

2. Couche photographique selon la revendication 1, caractérisée en ce que le rapport des moles d'ion nitrate aux moles de colorant est d'au moins 0,5.

3. Couche photographique selon l'une des revendications 1 et 2, caractérisée en ce que l'acide est présent dans le liant dans un rapport égal à jusqu'à 10 fois la quantité d'ion nitrate.

4. Couche photographique selon l'une des revendications 1 à 3, caractérisée en ce que le pH de la couche photographique est inférieur à 7,0. `

5. Couche photographique selon l'une des revendications 1 à 4, caractérisée en ce que le nitrate dans le liant est capable de libérer une quantité suffisante d'agent oxydant lorsqu'on le chauffe jusqu'à 160°C pendant 60 secondes.

6. Couche photographique selon l'une des revendications 1 à 5, caractérisée en ce que le nitrate comprend un nitrate métallique.

7. Couche photographique selon la revendication 6, caractérisée en ce que le nitrate comprend un nitrate métallique hydraté.

8. Couche photographique selon la revendication 7, caractérisée en ce que le nitrate est un sel hydraté d'un métal appartenant au groupe du zinc, cadmium, nickel, aluminium, fer, cuivre, magnésium, chrome, cobalt, bismuth, lanthané, gadolinium, thorium, zirconium et calcium.

9. Couche photographique selon l'une des revendications 1 à 8, caractérisé en ce qu'elle est insensible à la lumière.

10. Couche photographique selon l'une des revendications 1 à 9, caractérisée en ce que le colorant est présent en une quantité d'au moins 0,3% en poids par rapport au liant.

11. Couche photographique selon l'une des revendications 1 à 9, caractérisée en ce que le colorant est une matière colorante décolorable qui est présente à une concentration suffisante pour fournir une densité optique de transmission d'au moins 0,1 dans la région visible du spectre électromagnétique.

12. Couche photographique selon l'une des revendications 1 à 10, caractérisée en ce que le colorant est une matière colorante décolorable appartenant au groupe des méthines, indamines, anthraquinones, triarylméthanes, benzylidènes, monoazos, oxazines, azines, thiazines, xanthènes, indigoïdes, oxonols, cyanines, mérocyanines, phénols, naphthols et pyrazolones.

13. Couche photographique selon l'une des revendications 1 à 10, caractérisée en ce que le colorant est un leucocolorant appartenant au groupe des leucoviolet cristallisé, leucobleu malachite, leucovert malachite et 1(2-(1,3,3-triméthylindolyl))-2-(p-morpholinylphényl)-éthène.

## Patentansprüche

1. Eine Abbildungsschicht, umfassend ein polymeres Bindemittel und innerhalb dieses Bindemittels einen Leukofarbstoff oder bleichbaren Farbstoff und ein Nitratsalz, dessen Nitrat-Ion in einem Verhältnis von mindestens, 0,1 Mol/Mol Farbstoff vorhanden ist, wobei das Nitratsalz in dem Bindemittel in der Lage ist, beim Erhitzen auf 200°C für 60 Sekunden eine ausreichende Menge HN0₃, NO, N0₂ oder N₂0₄ als Oxidationsmittel freizusetzen, um den bleichbaren Farbstoff zu einer unterschiedlichen Farbe oder zum farblosen Zustand zu oxidieren oder den Leukofarbstoff zu einem gefärbten Zustand zu oxidieren, dadurch gekennzeichnet, daß eine Säure in dem Bindemittel vorhanden ist.

2. Abbildungsschicht gemäß Anspruch 1, in der das Molverhältnis Nitrat-Ion zu Farbstoff mindestens 0,5 beträgt.

3. Abbildungsschicht nach Anspruch 1 oder Anspruch 2, in der die Säure in dem Bindemittel in einem Verhältnis bis zur 10-fachen Menge des Nitrat-Ions vorhanden ist.

4. Abbildungsschicht nach einem der vorangehenden Ansprüche, in der der pH-Wert der Abbildungsschicht geringer als 7,0 ist.

5. Abbildungsschicht nach einem der vorangehenden Ansprüche, in der das Nitratsalz im Bindemittel in der Lage ist, die ausreichende Menge Oxidationsmittel beim Erhitzen auf 160°C für 60 Sekunden freizusetzen.

6. Abbildungsschicht nach einem der vorangehenden Ansprüche, in der das Nitratsalz ein Metall-Nitratsalz umfaßt.

7. Abbildungsschicht nach Anspruch 6, in der das Nitratsalz ein hydratisiertes Metall-Nitratsalz umfaßt.

8. Abbildungsschicht nach Anspruch 7, in der das Nitratsalz ein hydratisiertes Salz von Zink, Cadmium, Nickel, Aluminium, Eisen, Kupfer, Magnesium, Chrom, Kobalt, Wismut, Lanthan, Gadolinium, Thorium, Zirkonium oder Calcium ist.

9. Eine Abbildungsschicht nach einem der vorangehenden Ansprüche, die lichtunempfindlich ist.

10. Abbildungsschicht nach einem der Ansprüche 1- bis 9, in der der Farbstoff in einer Menge von mindestens 0,3 Gewichtsprozent des Bindemittels vorhanden ist.

11. Abbildungsschicht nach einem der Ansprüche 1 bis 9, in der der Farbstoff ein bleichbarer Farbstoff ist, der in einer Konzentration vorhanden ist, die ausreicht, um eine transmissive optische Dichte von mindestens 0,1 im sichtbaren Bereich des elektromagnetischen Spektrums zu ergeben.

12. Abbildungsschicht nach einem vorangehenden Anspruch, in der der Farbstoff ein bleichbarer Methin-, Indamin-, Anthrachinon-Triarylmethan-, Benzyliden, Monoazo-, Oxazin-, Azin-, Thiazin-, Xanthen-, Indigoid-, Oxonol-, Cyanin-, Merocyanin-, Phenol-, Naphthol- oder Pyrazolinfarbstoff ist.

13. Abbildungsschicht nach einem der Ansprüche 1 bis 10, in der der Farbstoff ein Leukokristallviolett-, Leukomalachitblau-, Leukomalachitgrün- oder 1-(2-(1,3,3-Trimethyiindoiyi))-2-(p-morphoiinyi- phenyl)-äthen-Leukofarbstoff ist.
